

No. 641,237.

Patented Jan. 9, 1900.

G. RUSSELL.  
METALLIC WALL COVERING.

(Application filed May 29, 1899.)

(No Model.)



WITNESSES:  
M. Hunter  
H. J. Devrie

Inventor,  
George Russell  
By O. D. Lewis  
Attest.

# UNITED STATES PATENT OFFICE.

GEORGE RUSSELL, OF MCKEESPORT, PENNSYLVANIA.

## METALLIC WALL-COVERING.

SPECIFICATION forming part of Letters Patent No. 641,237, dated January 9, 1900.

Application filed May 29, 1899. Serial No. 718,738. (No model.)

To all whom it may concern:

Be it known that I, GEORGE RUSSELL, a citizen of the United States of America, residing at McKeesport, in the county of Allegheny and State of Pennsylvania, have invented 5 certain new and useful Improvements in Metallic Wall-Coverings; and I do hereby declare the following to be a full, clear, and exact description thereof, reference being had 10 to the accompanying drawings, which form a part of this specification.

My invention relates to an improved metallic covering for walls and ceilings of rooms; and its object is to provide a covering for such 15 purpose that will be fireproof, impervious to the passage of germs and vermin, and which will also be proof against the deteriorating influence of dampness in any form.

I will now describe my invention, so that 20 others skilled in the art may make and use the same, reference being had to the accompanying drawings, forming part of this specification, in which—

Figure 1 is a perspective view of a roll or 25 package of my improved covering. Fig. 2 is an enlarged transverse sectional view of the same.

My improved covering is preferably made 30 as follows: I take a thin metallic sheet 1 of suitable length and width and apply to it on both sides one or more coatings 2 of plastic material, composed, preferably, of linseed-oil, shellac, and lead. The plate is then inserted 35 into a kiln or oven and subjected to an appropriate temperature—say from 300° to 400° Fahrenheit—for the purpose of “burning” the same. After the plate has been thus “burned” one or more coatings 3 of an enamel preparation, composed, preferably, of copal, 40 linseed-oil, and a suitable coloring material, are applied to the exterior surface of the plate and such coating or coatings are also baked in an oven or kiln heated to about the temperature above mentioned. The desired 45 ornamentation 4 in gold, bronze, enamel, &c., is then applied to the last-applied coating in any desired manner, preferably by means of the mechanism shown and described in Pat-

ent No. 524,736, granted to me August 21, 1894. The plate is then subjected to another 50 and final baking or burning operation, after which it is ready for use. The plates thus made may be applied to walls, ceilings, &c., in various ways and made to represent wall paper, either plain or paneled. 55

The foregoing method is my preferred method of making my improved covering; but it will be understood that other methods may be employed in making the same.

The advantages of my invention will be appreciated by those skilled in the art. It is economical to manufacture, durable, easy to keep clean, and is not liable to crack and break, as ordinary wall-coverings, and, as before mentioned, is proof against disease-germs, 65 fire, water, dampness, and vermin.

I claim—

1. As a new article of manufacture, a covering for walls and ceilings, composed of a plate of sheet metal having a coating on each 70 side, one of said coatings having a burned enameled surface.

2. As a new article of manufacture, a covering for walls and ceilings, composed of a plate of sheet metal having a coating on each 75 side, both of said coatings being burned and one having an enameled decorated surface.

3. As a new article of manufacture, a covering for walls and ceilings, composed of a plate of sheet metal having a burned coating 80 on each side.

4. As a new article of manufacture, a covering for walls and ceilings, composed of a plate of sheet metal having a burned primary coating on each side, a second burned enameled coating on one of the primary coatings; and decorations applied to the burned enameled coating. 85

In testimony whereof I have hereunto affixed my signature in the presence of two subscribing witnesses. 90

GEORGE RUSSELL.

Witnesses:

JOHN DOWNEY,  
JAMES J. CLOONAN.